

# UNITED STATES PATENT OFFICE.

JOHN HENRY JAMES, OF NASHVILLE, ARKANSAS, ASSIGNOR OF FIVE-EIGHTHS, BY DIRECT AND MESNE ASSIGNMENTS, TO WILLIAM F. ROBERTS, JR., AND FRANK D. THOMASON, OF CHICAGO, ILLINOIS.

## TANNING PROCESS.

SPECIFICATION forming part of Letters Patent No. 506,696, dated October 17, 1893.

Application filed January 18, 1892. Serial No. 418,420. (No specimens.)

*To all whom it may concern:*

Be it known that I, JOHN HENRY JAMES, a citizen of the United States, residing at Nashville, in the county of Howard and State of 5 Arkansas, have invented a new and useful Tanning Process, of which the following is a specification.

This invention relates to processes for tanning hides and compositions of matter used 10 in connection therewith, especially for manufacturing sole, harness or upper leather; and it has for its object to provide an improved process and compound whereby the resultant leather after being subjected to the treatment 15 embraced in this invention, will be soft and pliable, yet possessing a good body and color and having the characteristics of all good grades of leather.

With these and many other objects in view 20 which will readily appear to those skilled in the art as the nature of the invention is better understood, the same consists in the various steps and solutions used in connection therewith as will be hereinafter set forth and 25 claimed.

Before subjecting the hides to the tanning process proper, the same are subjected to several preliminary steps which particularly fit the same for being rapidly and effectively 30

acted upon by the tanning solution and process. After thoroughly soaking the green or dry hides in clear water and removing the flesh therefrom, the same are placed in a liming vat containing suitable proportions of lime, 35 lye soap or laundry soap. The hides remain immersed in this liming vat, being occasionally aired at suitable intervals, until the hair slips. The hides are now thrown into clear water and the hair worked out on the beam.

40 Then the same are skived and flattened out as evenly as possible. From the liming vat, the hides are next thrown into a bate pool containing one thousand gallons of water, and one half bushel of corn meal or one bushel of 45 wheat bran previously prepared by perfect fermentation. The bate pool solution is kept at a temperature of about 80° and frequently stirred. After remaining only for quite a short period in the bate pool, the hides are removed, 50 and all the remaining lime and short hair

taken therefrom and then washed. With these preliminaries the hides are ready for the tanning process.

The first tanning mixture which receives 55 the hides is composed of twenty pounds of Glauber's salts, twenty-two pounds of alum; twenty-five pounds of saltpeter, forty pounds of salt, and fifty pounds of gambier, which ingredients are thoroughly dissolved and added in solution to eight hundred gallons of clear 60 water. The hides are placed in this solution and for the first few days are handled every few hours. Thereafter from every six to twelve hours and continued until the hides are thoroughly tanned into leather. Having 65 subjected the hides to this tanning process proper the same are now again returned to the aforementioned solution to which has been added one hundred pounds of bark extract. The solution is then heated to blood heat, and 70 the hides therein are handled for forty-eight hours, at which time the leather will have a good body and color. The same is now to be well scoured, set, stuffed thoroughly, and finally allowed to dry. The leather thus produced 75 possesses all the essential qualities of and is particularly adapted for use as sole, harness or upper leather as originally pre- mised.

A fact of importance not to be overlooked 80 in connection with the improvements herein set forth, is that the bark extract is added to the cold solution of the tanning mixture before heat is applied with the hides immersed in such solution, and by practical experiment 85 it has been found that in order to secure the proper results the addition of the bark extract at this stage, and the heating up of the solution after the addition thereof, is absolutely necessary to secure the results claimed. 90 It is to be understood that the addition of the bark extract at this stage of the process not only serves to strengthen up the solution but also improves the color and renders a better 95 quality of leather, and it has been found that after the hides have been subjected to the action of the tanning mixture without the bark extract, the gelatine or glue in the hides is in the proper condition to receive the action of the tonic acid or bark extract, which to- 100

- gether with the mixture to which it is added, being heated up to a blood heat, makes the leather stiff, hard and impervious to the water, without breaking or cracking, which invariably occurs in processes where the leather is hardened up by introducing and applying hot oozee or liquor at any stage of the tanning, inasmuch as the combination of a warm or hot bark liquor with raw gelatine or glue, causes the pores of the hide or leather to open so that it becomes dry, crusty, and hard. These objectionable features of ordinary tanning processes are overcome by my improvement, and furthermore the results secured by me are designed only to be obtained in connection with the tanning mixture herein described.

Having thus described my invention, what I claim, and desire to secure by Letters Patent, is—

- 20 In the process of tanning hides, the im-

provement which consists in primarily depilating and bating, subjecting to the tanning action of a tanning mixture composed of Glauber's salts, alum, saltpeter, salt and gambier, introducing into such tanning mixture 25 a proportionate quantity of bark extract, while such tanning mixture is in a cool condition, re-immersing the hides in the new solution, raising the temperature of the latter with the hides therein to a blood heat, and 30 handling and manipulating the hides at intervals in the heated solution, substantially as set forth.

In testimony that I claim the foregoing as my own I have hereto affixed my signature in the presence of two witnesses.

JOHN HENRY JAMES.

Witnesses:

JAS. P. NEILLIVER,  
N. E. MULKEY.